# EUROPEAN PATENT APPLICATION

(11) **EP 4 779 050 A1**
(43) Date of publication of application: **22.07.2026**
(21) Application number: 24865927.8
(22) Date of filing: 17.05.2024
(51) Int. Cl.: C22C 38/38, C22C 38/24, C22C 38/34, C22C 38/00, C22C 38/26, C21D 8/02, C21D 9/46

(54) **STEEL MATERIAL AND METHOD FOR MANUFACTURING SAME**

(30) Priority: 13.09.2023 KR 20230122028
(71) Applicant: POSCO Co., Ltd, Gyeongsangbuk-do 37859 (KR)
(72) Inventor: LEE, Dong-Ho, Gwangyang-si, Jeollanam-do 57807 (KR)
(74) Representative: Meissner Bolte Partnerschaft mbB
(86) International application number: PCT/KR2024/095793
(87) International publication number: WO 2025/058488

(57) **Abstract**

The present invention relates to a steel material which can be used in various fields such as the energy industry and shipbuilding, and a method for manufacturing same.

## Description

### Technical Field

The present disclosure relates to a steel material which may be used in various fields such as the energy industry and shipbuilding, and a method for manufacturing the same.

### Background Art

The crude oil mining environment has become increasingly harsh, with oil becoming sour, containing a large amount of hydrogen sulfide, or the like, and accordingly, steel pipes and storage tank structures used to transport crude oil may require a material having excellent hydrogen embrittlement resistance. Accordingly, to mine and transport the crude oils, a material having excellent hydrogen embrittlement resistance and sufficient toughness and strength may be necessary to have resistance against external pressure during transportation.

As general high-strength carbon steel has a structure vulnerable to hydrogen embrittlement, known as hard spot, therein, and may thus be difficult to produce and have limited use. While various manufacturing methods and hard spot detection methods have significantly improved this issue, a large amount of high-strength structure may be necessary to increase strength fundamentally, and accordingly, it may be difficult to avoid hard spots, and thus difficult to obtain X80 grade or higher.

Also, in the case of a structure containing a large amount of steel, a military vessel such as a submarine, for example, the location of an adversary may be tracked by detecting changes in the magnetic field generated by interaction between the vessel and the Earth's magnetic field. Accordingly, when manufacturing a structure using steel which may maintain non-magnetism, the probability of detection may be significantly reduced.

When using general carbon steel to manufacture non-magnetic steel, a process called demagnetization, which periodically removes magnetism, may be performed. However, the operational time of the vessel may be reduced by the time for which the demagnetization is performed, and economic loss may also be incurred, which may not be preferable. Detailed description of present disclosure

### Technical problems to solve

An embodiment of the present disclosure is to provide a steel material having excellent non-magnetic properties and excellent hydrogen embrittlement resistance, and a method for manufacturing the same.

The subject matter of the present disclosure may not be limited to the matters described above. Additional matters of the present disclosure are described throughout the specification, and those skilled in the art to which the present disclosure pertains will have no difficulty in understanding the additional matters of the present disclosure from the descriptions described in the specification of the present disclosure.

### Solution to Problem

According to an embodiment of the present disclosure, a steel material includes, by weight%, manganese (Mn): 13.0 to 25.0%, carbon (C): in a range satisfying 10×[C]+[Mn]≥20.0, chromium (Cr): 5.0% or less (excluding 0%), vanadium (V): 1.5% or less (excluding 0%), and a balance of Fe and inevitable impurities,

wherein a microstructure includes 95% or more (100% include) of austenite and 5% or less (0% include) of carbides by area%.

The steel material includes one or more of niobium (Nb): 1% or less, silicon (Si): 5% or less and nitrogen (N): 1% or less.

An average grain size of the austenite is 5 to 200 µm.

The steel material includes 10 or more carbides having a size of 100 nm or less, observed per 100 nm*100 nm unit area.

The steel material has a crack length ratio (CLR) of 10 or less in a hydrogen-induced cracking (HIC) test, defined by equation 1 below:

$CLR \left(Crack Length Ratio, %\right) = \sum \left(a/W\right) * 100$
where a indicates a length of a single crack, and W indicates a width of a sample.

The steel material has a permeability of less than 1.01 after 30% of plastic deformation.

According to an embodiment of the present disclosure, a steel material includes heating a steel slab including, by weight%, manganese (Mn): 13.0 to 25.0%, carbon (C): in a range satisfying 10×[C]+[Mn]≥20.0, chromium (Cr): 5.0% or less (excluding 0%), vanadium (V): 1.5% or less (excluding 0%), and a balance of Fe and inevitable impurities, at 1000 to 1300°C;
finishing hot-rolling the heated steel slab at 800 to 1050°C; and
cooling the heated steel slab to a temperature within a range of 500°C or lower at a cooling rate of 10°C/s or higher after hot rolling.

The steel slab includes one or more of niobium (Nb): 1% or less, silicon (Si): 5% or less and nitrogen (N): 1% or less.

The heating satisfies a heating time of equation 2 below: [Equation 2] heating time (min) ≥ 1/4 × slab thickness (mm) + 30 min.

### Advantageous Effects of Invention

According to an aspect of an embodiment of the present disclosure, provided is a steel material which may be used in a structure requiring excellent hydrogen embrittlement resistance properties, such as a ship hull requiring excellent non-magnetic properties, or a steel pipe or a facility transporting crude oil having a high content of hydrogen sulfide.

The various beneficial advantages and effects of the present disclosure are not limited to the above-described contents, and will be more easily understood in the process of describing the specific embodiments of the present disclosure.

### Brief Description of Drawings

FIG. 1 schematically illustrates a sample for calculating a crack length ratio (CLR) during a hydrogen-induced cracking (HIC) test.
FIG. 2 illustrates an EPMA image (a) and a transmission electron microscope (TEM) image (b) from observing a microstructure of invention example 1 in embodiment 1.
FIG. 3 illustrates a transmission electron microscope (TEM) image of comparative example 2 in embodiment 1.
FIG. 4 illustrates an optical microscopic image from observing an internal structure of a steel slab to which different heating times are applied in embodiment 2.

### Best Mode for Invention

The terminology used in this specification is intended to describe the present disclosure and is not intended to limit the present disclosure. Also, the singular forms used herein may also include plural forms, unless otherwise indicated.

The term "including" used herein specifies a component and does not exclude the presence or addition of other components.

Unless otherwise indicated, the entirety of terms, including technical and scientific terms, used herein have the same meaning as commonly understood by a person of ordinary skill in the art to which the present disclosure pertains. Terms defined in the dictionary are to be interpreted to have meanings consistent with the relevant technical document and the present disclosure.

First, an example of the steel material of the present disclosure will be described in detail. In the description below, the alloy composition and range of the steel material will be described. The content of the alloy composition described below may refer to weight% unless otherwise indicated.

### Manganese (Mn): 13.0 to 25.0%

Mn may be important in stabilizing austenite. The steel material may include 13.0% or more of Mn to stabilize austenite. When the Mn content is less than the above content, epsilon (ε) martensite, a metastable phase, may be formed, and may be easily transformed to alpha martensite through deformation-induced transformation at ultra-low temperature, such that toughness may not be ensured. To suppress the formation of epsilon (ε) martensite, austenite may be stabilized by increasing the carbon (C) content. However, in this case, the large amount of carbides may be precipitated, such that properties, specifically toughness, may be rapidly deteriorated. Accordingly, the Mn content may be 13.0% or more. A preferable Mn content may be 15% or more, and a more preferable Mn content may be 18% or more. The excessive Mn content may lower the corrosion rate of the steel material, and may not be economical. Accordingly, the Mn content may be 22% or less, preferably. More preferably, the Mn content may be 20% or less.

### Carbon (C): 10 × [C] + [Mn] ≥ 20.0

C may stabilize austenite and may increase strength. In particular, C may lower Ms or Md, transformation points from austenite to epsilon or alpha martensite, during cooling or processing processes. Accordingly, C may effectively contribute to the stabilization of austenite. When the C content is insufficient, austenite stability may be insufficient, such that it may be difficult to obtain stable austenite at ultra-low temperature. Also, deformation-induced transformation into epsilon or alpha martensite may easily occur under external stress, which may reduce toughness or strength of the steel. Accordingly, the C content may be 0.01% or more. On the other hand, when the C content is excessive, toughness of the steel may deteriorate rapidly due to carbide precipitation, and strength of the steel may increase excessively, which may reduce workability.

The inventors of the present disclosure have conducted in-depth research on the relative behavior between the C and Mn contents in relation to carbide formation, and have concluded that determining the relative content relationship between C and Mn may effectively promote austenite stabilization while controlling the amount of carbide precipitation. C may be formed by carbon, but C does not independently influence carbide formation, and may interact with Mn and other alloying elements and may influence carbide formation.

To stabilize austenite, it may be preferable to maintain the value of 10×[C]+[Mn] (where [C] and [Mn] indicate the content of each element in weight%) at 20.0 or more, assuming that other elements may meet the ranges specified in the present disclosure. When 10×[C]+[Mn] is less than 20.0, the stability of austenite may decrease, leading to deformation-induced transformation and accordingly, impact toughness of the steel may degrade. Also, when deformation-induced transformation occur, alpha-prime (α') martensite having a BCC structure may be formed in addition to non-magnetic austenite, which may increase permeability. Thus, 20.0 or more may be preferable.

### Chromium (Cr): 5.0% or less (excluding 0%)

Cr may also be an austenite-stabilizing element, and may stabilize austenite within an appropriate amount, thereby improving low-temperature impact toughness of steel, and by being dissolved in austenite, Cr may increase strength of the steel. Also, Cr may effectively contribute to improving corrosion resistance of steel. Accordingly, in the present disclosure, Cr may be added as an essential element. A preferable lower limit of the Cr content may be 1%, and a more preferable lower limit of the Cr content may be 2%.

However, Cr may be a carbide-forming element, and particularly, Cr may form carbides at austenite grain boundaries, thereby reducing the low-temperature impact toughness of steel. Also, when the Cr content exceeds a specific level, excessive carbide may be precipitated in the weld heat-affected zone (HAZ), which may deteriorate ultra-low temperature toughness. Accordingly, an upper limit of the Cr content may be 5.0%. A preferable upper limit of the Cr content may be 4%.

### Vanadium (V): 1.5% or less (excluding 0%)

Vanadium (V) may form carbides by combining with carbon, may inhibit grain growth in the austenite structure and may delay recrystallization, thereby contributing to strength enhancement. Even when a trace of amount of V is added, grain growth in the austenite structure may be obtained. Thus, a lower limit of the V content in the present disclosure may be limited to a range excluding 0%. As the formation of fine carbides exceeding a specific fraction may more effectively contribute to the strength enhancement of the steel material, in the present disclosure, a preferable lower limit of the V content may be limited to 0.1% in consideration of the precipitation strengthening caused by carbide formation. When V is excessively added, it may be impossible to completely dissolve coarse carbides formed during the steelmaking process during reheating, and coarse carbide may remain in subsequent processes, which may degrade properties. Also, as V is an expensive element, adding excessive amount of V may not be economically preferable. Accordingly, in the present disclosure, an upper limit of the V content may be limited to 1.5%, and a preferable upper limit of V content may be 1%.

The steel material may further include one or more of Nb: 1% or less, Si: 5% or less, and N: 1% or less.

### Niobium (Nb): 1% or less

Nb may form NbC carbides by combining with carbon, and may inhibit grain growth in the austenite structure and may increase the recrystallization temperature, thereby increasing rolling capacity in the non-recrystallized region during the steel material manufacturing process, and contributing to strength enhancement. Even when Nb is added in a small amount, the grain growth effect in the austenite structure may be further obtained, but in the present disclosure, Nb may not be essential. However, as the formation of a specific fraction or more of fine NbC carbides may more effectively contribute to the strength enhancement of the steel material, in the present disclosure, a preferable lower limit of the Nb content may be 0.01%, considering the precipitation strengthening caused by carbide formation. When Nb is added excessively, coarse carbides formed during the steelmaking process may be vulnerable to external force in the continuous tank process, which may cause cracks, and may deteriorate properties. Also, when the large amount of Nb is added, as a large amount of coarse carbides may precipitate in the weld heat-affected zone, which may reduce impact toughness. Accordingly, in the present disclosure, an upper limit of the Nb content may be limited to 1%.

### Silicon (Si): 5% or less

Silicon may improve castability of molten steel and, when added to austenitic steels, silicon may effectively increase strength by dissolving in the steel. Silicon may also affect the activity of carbon in steel, effectively suppressing carbide formation and increasing toughness. However, when added in excess of 5%, stacking fault energy may be decreased, which may promote twinning and may reduce toughness due to increased strength. Thus, an upper limit may be limited to 5%, preferably. A preferable upper limit of the silicon (Si) content may be 3%, and a more preferable upper limit of the silicon (Si) content may be 2.5%. Preferably, a lower limit of the silicon (Si) content may be 0.1%, and a more preferable lower limit of the silicon (Si) content may be 0.3%.

### Nitrogen (N): 1% or less

N may stabilize austenite and may improve toughness along with carbon, and N may be particularly advantageous for enhancing strength through solid-solution strengthening, similarly to carbon. In particular, N is well known as an element effectively increasing stacking fault energy and promoting slip. However, when added in excess of 1%, coarse nitrides may be formed, which may degrade the surface quality and properties of the steel material. Thus, preferably, an upper limit may be limited to 1 wt%. A preferable upper limit of the nitrogen (N) content may be 0.5%, and a more preferable upper limit of the nitrogen (N) content may be 0.2%. Preferably, a lower limit of the nitrogen (N) content may be 0.005%, and a more preferable lower limit of the nitrogen (N) content may be 0.007%.

The steel material in the present disclosure may include iron (Fe) and inevitable impurities unintentionally included during a general manufacturing process. These impurities may be readily apparent to a person skilled in the art of steel manufacturing, and thus, the description thereof is not provided in this specification.

The steel material may include 95% or more austenite in a microstructure by area%. Preferably, the fraction may include 97% or more, and may include a 100% austenite fraction.

Meanwhile, the steel material may include carbides to prevent a decrease in impact toughness. Examples of carbides may include vanadium carbide (VC). The carbides may be present in grains of the steel or at grain boundaries, and may be formed in sizes of several tens of nanometers or less. According to the observation using a transmission electron microscope (TEM), carbides may include 10 or more carbides measuring 100 nm or less per 100 nm x 100 nm unit area. An upper limit thereof is not particularly limited, but may be 20,000 or less.

In steel materials, austenite may be an unstable structure at room temperature. Generally, to maintain austenite, which is stable at high temperature, at room temperature, austenite-stabilizing elements may be added. Even when austenite is obtained at room temperature, by further cooling or processing, austenite may be transformed into epsilon martensite or alpha martensite, which may be varied depending on the alloy composition, cooling temperature, and processing amount. As austenitic steel materials may generally undergo cold working for structural forming, when a rolled material is produced, even when the microstructure is austenitic, phase transformation may occur by processing during manufacturing a structure. When weak epsilon or alpha martensite is formed by phase transformation, impact toughness may be deteriorated and non-magnetic properties may deteriorate.

Austenite in the steel material of the present disclosure may have an average grain size of 5 to 200 µm. When the average austenite grain size exceeds 200 µm, due to austenite coarsening, strength may decrease. Also, the deformation-induced transformation temperature may increase, transformation to epsilon martensite or martensite may easily occur during processing, which may reduce impact toughness. When the average austenite grain size is less than 5 µm, strength may excessively increase, such that toughness may decrease. Preferably, a lower limit of the average austenite grain size may be 7 µm, or more preferably, 10 µm. More preferably, an upper limit of the average austenite grain size may be 180 µm, or more preferably, 150 µm.

The steel material of the present disclosure may have an impact toughness of 30 J or more after a Charpy impact test at -100°C.

The inventors of the present disclosure have found that hydrogen embrittlement resistance may be a key factor in ensuring safety when applied to sour environment. A steel material having excellent sour resistance according to an embodiment of the present disclosure may have a yield strength of 500 MPa or more and an elongation of 20% or more. As strength of a steel material increases, impact toughness may decrease. Specifically, as for the steel material of the present disclosure, when yield strength is excessively high, it is highly likely that target impact toughness may not be ensured. Accordingly, an upper limit of the room temperature yield strength in the present disclosure may be 900 MPa.

Also, a steel material having excellent resistance against sour according to an embodiment of the present disclosure may have a crack length ratio (CLR) of 10 or less during a hydrogen-induced cracking (HIC) test, and a preferable crack length ratio (CLR) may be 5 or less, and a more preferable crack length ratio (CLR) may be 2 or less.

Hereinafter, the crack length ratio (CLR) during the hydrogen-induced cracking (HIC) test will be described in greater detail.

The hydrogen-induced cracking (HIC) test may be performed by immersing a sample in an acidic solution (5% NaCl + 0.5% CH₃COOH) saturated with H₂S gas, maintaining the solution for 96 hours, and observing the location of crack initiation. Specifically, as illustrated in FIG. 1, a cross-section of a sample having a constant width (w) and thickness (T) is observed, and the crack length (a) may be measured at the point of crack initiation. The crack length ratio (CLR) may be derived from the average of these values. The equation for calculating the crack length ratio (CLR) may be Equation 1 as below. In FIG. 2, the symbol b may indicate the crack thickness.$CLR \left(Crack Length Ratio, %\right) = \sum \left(a/W\right) * 100$

In equation 1, "a" represents the length of a single crack, and "W" represents the width of the sample.

As the crack length ratio (CLR) decrease, the resistance to hydrogen-induced cracking may be more excellent. In particular, when crack length ratio (CLR) is 10 or less, or preferably 5 or less, excellent resistance to hydrogen-induced cracking may be ensured even in severe oxidizing environment.

The permeability of the steel material of the present disclosure may be maintained at 1.01 or less even with 30% plastic deformation.

In the description below, an example of a method of manufacturing a steel material of the present disclosure will be described in detail.

The manufacturing method may include a process of heating, hot rolling and cooling a steel slab having the aforementioned alloy composition, which will be described in greater detail below.

First, the steel slab having the aforementioned alloy composition may be heated at 1000 to 1300°C. When the slab heating temperature is lower than 1100°C, the alloy components may not be re-dissolved and homogenized, or it may take a long time to reach the target temperature at the center of the slab. When the slab heating temperature exceeds 1300°C, partial melting may occur in the slab alloy component segregation zone, or severe surface oxidation may occur. More preferably, a lower limit of the slab heating temperature may be 1030°C, even more preferably, 1070°C, and most preferably, 1100°C. More preferably, an upper limit of the slab heating temperature may be 1250°C, even more preferably 1230°C, and most preferably 1200°C.

Also, preferably, the heating time during the heating process may satisfy equation 2 below. Equation 2, the heating time, may need to be satisfied such that the steel slab may go through sufficient soaking. An upper limit of the heating time is not limited, but may be preferably 5 hours or less, and more preferably, 4 hours or less. [Equation 2] Heating time (minutes) ≥ 1/4 × slab thickness (mm) + 30 minutes

Thereafter, the heated slab may be finishing hot-rolled at 800 to 1050°C, thereby obtaining a hot-rolled steel sheet. When the finishing hot-rolling temperature is lower than 800°C, rolling may difficult due to the high-temperature strength of the material, and excessive rolling may be carried out in the non-recrystallized region, such that strength of the material may increase excessively, which reduces impact toughness. When the finishing hot-rolling temperature exceeds 1050°C, austenite may be coarsened, such that strength may decrease. More preferably, a lower limit of the finishing hot-rolling temperature may be 820°C, and even more preferably, 850°C. Carbides, especially VC, may be formed near the finishing temperature, which may increase yield strength through precipitation strengthening. In this case, VC may be formed in the grains and grain boundaries with a size of tens of nm or less, and may be identified, for example, in the image of FIG. 2. More preferably, an upper limit of the finishing hot-rolling temperature may be 1030°C, more preferably 1000°C, and most preferably 980°C. Meanwhile, the reduction ratio during hot rolling may be applied within an appropriate range depending on the target sheet thickness. As a non-limiting example, the final thickness of the hot-rolled steel sheet may range from 5 to 50 mm.

Thereafter, the hot-rolled steel sheet may be rapidly cooled to a temperature within a range of 500°C or lower at a cooling rate of 10°C/s or higher. When the cooling rate is lower than 10°C/s or the cooling end temperature exceeds 500°C, excessive cementite precipitation may occur, such that impact toughness may degrade. Since most of the cementite formed during cooling is formed along grain boundaries, it may be preferable to suppress the formation of cementite as much as possible by appropriately controlling the cooling rate and the cooling end temperature. Accordingly, the cooling rate in the present disclosure may be 10°C/s or higher, the cooling end temperature may be 500°C or lower, and a preferable cooling rate may be 15°C/s or higher, and a preferable cooling end temperature may be 450°C or lower. Also, in the present disclosure, an upper limit of the cooling rate is not particularly limited, but an upper limit of the cooling rate may be limited to 120°C/s in consideration of factors such as distortion of the steel sheet shape and the economical aspect.

Hereinafter, embodiments of the present disclosure will be described. It should be understood that various modifications to the embodiments described below may be made for those skilled in the art, without departing from the scope of the present disclosure. The embodiments described below are intended to facilitate understanding of the present disclosure. The scope of the present disclosure should not be limited to the embodiments described below, but should be determined by the claims described below and equivalents thereof.

### (Embodiment 1)

A 250 mm thick slab having the alloy composition (unit: weight%, with the remainder of Fe and inevitable impurities) as in table 1 was prepared, and the slab was heated and hot rolled as described in Table 2, thereby manufacturing a steel material.

The microstructure and properties of the manufactured steel material were measured, and the results are listed in Table 2.

The microstructure was measured at room temperature using an optical microscope.

The average austenite grain size was measured by obtaining a microstructure image using an optical microscope, and performing image analysis.

The room-temperature yield strength was measured using a uniaxial tensile test, and the Charpy impact energy (CVN) value was measured by obtaining a standard sample of the steel material in accordance with ASTM A370, and cooling to -100°C, and the impact energy was measured according to ASTM standards.

**[Table 1]**

| Steel type | Alloy composition (weight%) | | | | | | |
|---|---|---|---|---|---|---|---|
| | Mn | 10X[C]+[Mn]≥20.0 | Cr | V | Nb | Si | N |
| A | 18.05 | 24.05 | 3.14 | 0.51 | 0.03 | 0.38 | 0.011 |
| B | 16.2 | 23.2 | 2.85 | 0.45 | 0.02 | - | - |
| C | 17 | 20.0 | 2.45 | 0.55 | 0.03 | 0.85 | - |
| D | 21.1 | 22.1 | 3.57 | 0.32 | 0.01 | - | 0.15 |
| E | 19.3 | 24.3 | 4.75 | 0.28 | 0.1 | 1.05 | - |
| F | 18.5 | 18.6 | 3.11 | 0.01 | 0.038 | - | - |
| G | 17.3 | 19.3 | 2.68 | 0.14 | 0.01 | - | - |
| H | 13.1 | 14.6 | 11.2 | 0.89 | 0.005 | - | - |
| I | 24.5 | 28.3 | 0.92 | 0 | 0.01 | - | - |
| J | 14.4 | 17.5 | 1.08 | 0.18 | 0.0001 | - | - |
| K | 15.2 | 18 | 2.89 | 0.8 | 0.031 | - | - |

**[Table 2]**

| Classification | Steel type | Slab heating temperature (°C) | Finishing hot rolling (°C) | Steel material thickness (mm) | Microstructure (area%) | Austenite Average Grain Size ( µm) | Room temperature yield strength (MPa) | Charpy impact energy (J, @-100°C) |
|---|---|---|---|---|---|---|---|---|
| Inventive exampl e 1 | A | 1185 | 913 | 18 | 100%γ | 43 | 623 | 78 |
| Inventive example 2 | B | 1180 | 910 | 20 | 100%γ | 40 | 580 | 84 |
| Inventive example 3 | C | 1202 | 917 | 30 | 100%γ | 37 | 554 | 88 |
| Inventive example 4 | D | 1195 | 897 | 30 | 100%γ | 52 | 551 | 89 |
| Inventive example 5 | E | 1208 | 928 | 17 | 100%γ | 64 | 642 | 73 |
| Comparative example 1 | F | 1185 | 915 | 12.7 | 18%ε+11%M+71%γ | 61 | 347 | 26 |
| Comparative example 2 | G | 1179 | 942 | 20 | 5%ε+7%M+88%γ | 52 | 480 | 22 |
| Comparative example 3 | H | 1190 | 918 | 22 | 90%γ+10%carbide | 57 | 254 | 27 |
| Comparative example 4 | I | 1205 | 916 | 17 | 26%ε+17%M+57%γ | 47 | 430 | 14 |
| Comparative example 5 | J | 1198 | 920 | 28 | 82%γ+18%carbide | 86 | 373 | 20 |
| Compar ative example 6 | K | 1186 | 1186 | 34 | 20%ε+13%M+67%γ | 215 | 277 | 16 |

(In table 2, γ: austenite, M: α'-martensite, ε: ε-martensite, and here, carbide indicates bulk carbide such as chromium carbide.)

As for inventive examples 1 to 5, which satisfied the alloy composition and the manufacturing conditions of the present disclosure, the desired microstructure and average austenite grain size targeted in the present disclosure were ensured, thereby ensuring excellent properties.

(a) of FIG. 2 is an EPMA image of carbides within the structure of inventive example 1, confirming VC carbides. According to (a) of FIG. 2, it may be confirmed that inventive example 1 included 10 or more VCs of 100 nm or less per unit area. (b) is a transmission electron microscope (TEM) image, confirming VC carbide (circled) formed around grain boundaries.

FIG. 3 is a transmission electron microscope (TEM) image of comparative example 2, and the grain boundary (indicated by a dotted line) is identified. In FIG. 3, carbides were thickly formed at the grain boundaries, such that C was exhausted, and C to precipitate VC carbides was insufficient in the grain, and VC carbide was not observed in the structure.

As for comparative examples 1 to 6, which did not satisfy the alloy composition or the microstructure of the present disclosure, the microstructure or the average austenite grain size targeted in the present disclosure was not ensured, exhibiting low properties.

Meanwhile, permeability and CLR were measured for some of the samples according to the plastic deformation rate, and the results are listed in tables 3 and 4 below.

Permeability may be represented as relative permeability, which is the ratio of permeability in vacuum to permeability in a specific atmosphere. In the embodiment, the relative permeability (µ), which is the permeability ratio in vacuum and atmosphere, was measured using a paramagnetic measuring device.

The hydrogen-induced cracking (HIC) test may be performed by immersing a sample in an acidic solution (5% NaCl + 0.5% CH₃COOH) saturated with H₂S gas, maintaining for 96 hours, and observing the location of crack initiation. A cross-section of a sample with a constant width (W) and thickness (T) was observed, and the crack length (a) was measured at the point of crack initiation. The crack length ratio (CLR) may be derived from the average of these values. The equation for calculating the crack length ratio (CLR) is as in Equation 1 below.$CLR \left(Crack Length Ratio, %\right) = \sum \left(a/W\right) * 100$

a in equation 1 indicates the length of a single crack, and W may indicate the width of the sample.

**[Table 3]**

| Classification | Steel type | Plastic deformation rate (%) | Permeability |
|---|---|---|---|
| Inventive example 1 | A | 0 | 1.001 |
| | | 10 | 1.00317 |
| | | 20 | 1.0045 |
| | | 30 | 1.00433 |
| Inventive example 2 | B | 0 | 1.001 |
| | | 10 | 1.0035 |
| | | 20 | 1.0039 |
| | | 30 | 1.0041 |
| Comparative example 3 | H | 0 | 1.125 |
| | | 10 | 1.1945 |
| | | 20 | 1.3675 |
| | | 30 | 2.18633 |
| Comparative example 5 | J | 0 | 1.235 |
| | | 10 | 1.314 |
| | | 20 | 1.672 |
| | | 30 | 2.363 |

**[Table 4]**

| Classification | Steel type | CLR (%) |
|---|---|---|
| Inventive example 1 | A | 0.0 |
| Inventive example 2 | B | 0.0 |
| Comparative example 1 | F | 11.3 |
| Comparative example 6 | K | 14.7 |

According to tables 3 and 4, as for inventive examples 1 and 2 according to the present disclosure, even when the plastic deformation rate was 30% or more, a permeability was 1.01 or less, such that excellent non-magnetic properties and hydrogen embrittlement resistance were ensured. However, comparative examples 3 and 5 exhibited poor non-magnetic properties, and comparative examples 1 and 6 exhibited deteriorated hydrogen embrittlement resistance.

### (Embodiment 2)

In embodiment 1, a steel material was manufactured using steel Type A under the same conditions as inventive example 1. However, the heating time during the steel slab heating process was varied to 30 minutes, 1 hour, 2 hours, and 3 hours. An optical microscope image of the steel slab after heating is presented in FIG. 4. (a) and (b) of FIGS. 4 are the cases in which the heating time was 30 minutes and 1 hour, respectively, and the heating time condition of equation 2 was not satisfied. Accordingly, a large amount of carbide was formed in the steel slab, and due to the lack of re-dissolved C, the formation of VC carbide in the final steel material was not able to be expected. Also, when coarse carbide (bulk carbide) is formed in the steel slab and C is consumed in the coarse carbide, the austenite stability of the microstructure may decrease, and the large amount of coarse carbide may be contained in the final rolled steel material, such that impact toughness may decrease rapidly. [Equation 2] Heating time (min) ≥ 1/4 × slab thickness (mm) + 30 min

(c) and (d) of FIG. 4 shows images of a steel slab of which the heating times were 2 and 3 hours, respectively, and which satisfied the heating time condition of equation 2, thereby having gone through sufficient soaking. Redissolution was sufficiently carried out, such that the formation of VC carbides and other materials in the final steel material may be expected.

## Claims

1. A steel material, comprising:
by weight%, manganese (Mn): 13.0 to 25.0%, carbon (C): in a range satisfying 10×[C]+[Mn]≥20.0, chromium (Cr): 5.0% or less (excluding 0%), vanadium (V): 1.5% or less (excluding 0%), and a balance of Fe and inevitable impurities,
wherein a microstructure includes 95% or more (100% include) of austenite and 5% or less (0% include) of carbides by area%.

2. The steel material of claim 1, wherein the steel material comprises one or more of niobium (Nb): 1% or less, silicon (Si): 5% or less and nitrogen (N): 1% or less.

3. The steel material of claim 1, wherein an average grain size of the austenite is 5 to 200 µm.

4. The steel material of claim 1, wherein the steel material includes 10 or more carbides having a size of 100 nm or less, observed per 100 nm*100 nm unit area.

5. The steel material of claim 1, wherein the steel material has a crack length ratio (CLR) of 10 or less in a hydrogen-induced cracking (HIC) test, defined by equation 1 below: $CLR \left(Crack Length Ratio, %\right) = \sum \left(a/W\right) * 100$ where a indicates a length of a single crack, and W indicates a width of a sample.

6. The steel material of claim 1, wherein the steel material has a permeability of less than 1.01 after 30% of plastic deformation.

7. A method for manufacturing a steel material, the method comprising:
heating a steel slab including, by weight%, manganese (Mn): 13.0 to 25.0%, carbon (C): in a range satisfying 10×[C]+ [Mn]≥20.0, chromium (Cr): 5.0% or less (excluding 0%), vanadium (V): 1.5% or less (excluding 0%), and a balance of Fe and inevitable impurities, at 1000 to 1300°C;
finishing hot-rolling the heated steel slab at 800 to 1050°C to obtain a hot-rolled steel sheet; and
cooling the hot-rolled steel sheet to a temperature within a range of 500°C or lower at a cooling rate of 10°C/s or higher after hot-rolling.

8. The method of claim 7, wherein the steel slab comprises one or more of niobium (Nb): 1% or less, silicon (Si): 5% or less and nitrogen (N): 1% or less.

9. The method of claim 7, wherein the heating satisfies a heating time of equation 2 below: heating time (min) ≥ 1/4 × slab thickness (mm) + 30 min.
